

May 10, 1932.

W. W. POUNDSTONE

1,857,213

PROCESS OF MAKING OPTICAL DISKS

Filed Feb. 28, 1930 2 Sheets-Sheet 1

Fig. 1.



Fig. 2.



Fig. 3.



Fig. 4.

INVENTOR  
W. W. Poundstone  
by  
James G. Bradley  
atty

May 10, 1932.

W. W. POUNDSTONE

1,857,213

PROCESS OF MAKING OPTICAL DISKS

Filed Feb. 28, 1930

2 Sheets-Sheet 2



INVENTOR  
W. W. Poundstone  
by  
James C. Bradley  
atty

## UNITED STATES PATENT OFFICE

WILLIAM W. FOUNDRY, OF CHARLEROI, PENNSYLVANIA, ASSIGNOR TO PITTSBURGH PLATE GLASS COMPANY, A CORPORATION OF PENNSYLVANIA

## PROCESS OF MAKING OPTICAL DISKS

Application filed February 28, 1930. Serial No. 432,066.

The invention relates to a process of making optical disks from rectangular blanks (blanks rectangular in cross section) and particularly to the treatment of the blanks so that the lower surfaces of the disks which ordinarily are somewhat rough and hazy are smooth and clear, and so that the blanks have no tendency to stick in the molds. In preparing blanks for pressing heretofore, it has been the practice to carry them through a furnace or oven to bring them to a plastic state and then press them into molds. In order to keep the blanks from sticking to the support on which they rest in the furnace, it has been the practice to use powdered clay, pumice or graphite on such support. This powdered material sticks to the bottoms of the blanks and produces a discoloration or haze when they are pressed. It has also been found necessary to carbonize the mold to prevent the blanks from sticking therein. In the practice of my invention, the use of the powdered materials in the manner above referred to, which clouds the surfaces of the disks, is avoided, and the requirement for carbonizing the molds is avoided.

As a substitute for the powdered material, I employ a mixture of graphite and machine oil which is applied to the lower side of the blanks, preferably in the form of a spray before the blanks are placed in the furnace. This prevents the blanks from sticking either to the hearth of the furnace or to the molds during the pressing operation. The graphite mixture leaves the disks smooth and substantially free from any haze or discoloration. The practice of the invention is illustrated in the accompanying drawings, where-

in: Figure 1 is a transverse section through a furnace in which the blanks are heated preliminary to pressing. Fig. 2 is a longitudinal section through the furnace. Fig. 3 is a transverse section through a furnace of the rotary type. Fig. 4 is a longitudinal section through such furnace. Figs. 5 and 6 are perspective views of the rectangular blanks from which the disks are pressed. Fig. 7 is a transverse section through one of the blanks. Fig. 8 is a section through one of

the blanks and its carrier after such blank has been made plastic in the furnace. And Fig. 9 is a vertical section through the mold in which the blank is pressed.

The furnace shown in Figs. 1 and 2 is preferably of the straight-away type and comprises an elongated chamber 1 heated from the burners 2 and provided with an endless carrier for the blanks in the form of a series of plates 3 of heat resisting metal, such as "calite", carried at their ends by the roller chains 4, 4. These roller chains are mounted upon guides 5, 5 located outside the walls of the furnace and carried by frames 6, 6.

The glass blanks may be of the elongated rectangular type 7, such as shown in Fig. 5, or of the square type 8, such as shown in Fig. 6. When the elongated type, such as 7, is used, a plurality of disks are punched from such blank at one time in the molding operation, the apparatus including in such case a series 70 of molds placed side by side and a series of plungers. The blanks are pressed into molds 9, such as those shown in Fig. 9, such molds being provided with cavities 10 for receiving the heated blank. A plunger, not shown, is used for pressing the blank into the mold, the mold and plunger construction being 75 one well-known in the art.

Before the blanks are placed in the furnace 80 for heating, their lower sides are covered with the coatings 11. This coating is preferably a mixture of machine oil and graphite, although any liquid may be used as a carrier for the graphite which is readily oxidized when the blank is heated. For instance, turpentine may be substituted for the oil, if desired. The coating may be applied by spraying, dipping or brushing, but the spray method is preferred as this gives a very light coating 85 which is uniform throughout. A non-uniform coating, such as ordinarily produced by applying a liquid with a brush tends to show lines on the surface of the blank after the pressing operation. When the coating is 90 sprayed on the lower face of the blank, some of the material works around the edges onto the narrow surfaces of the blank, as indicated in Figs. 5 and 6. This is a desirable condition, since the blank is inclined to flatten 95 100

down somewhat when heated in the furnace, as indicated in Fig. 8, and if the coating did not extend over the side edges of the blank, the glass would touch the carrier at its extreme edges and tend to stick thereto. After the blanks are coated on their lower sides, they are placed on the plates 3 in the furnace and carried therethrough, being heated until they are somewhat plastic so that they can be pressed. During this period of heating, the graphite coating 11 on the blanks prevents their sticking to the plates 3. After they are properly heated, the blanks are placed in molds 9 and pressed from rectangular to disk form, the coated face of the blank, during this pressing operation, engaging the lower surface of the mold 9. The coating on the blanks presents an advantage in connection with this pressing operation in that it prevents the blanks from sticking in the molds as they would otherwise have a tendency to do after the molds become highly heated. The use of the graphite mixture, therefore, prevents any sticking throughout the entire operation and the lower surfaces of the disk thus produced are relatively smooth and free from any discoloration, so that the blanks may be readily inspected and the quality of the glass determined.

Figs. 3 and 4 illustrate a modified form of furnace, such furnace being of the circular type provided with an annular clay hearth 12 whose upper surface constitutes the floor of the chamber 13 and which is suitably rotated to carry the blanks through the furnace. This furnace is shown as heated with burners 14 the same as in the other type of construction. The blanks 8 might be supported directly upon the clay hearth 12, but a calite plate 15 is preferably provided to constitute the top of the hearth 12 and receive the blanks.

The solid material used in the mixture is preferably graphite, as this gives the best results so far attained, but it is possible to use substitutes, which approximate the results secured with graphite, such as finely powdered mica, sand and clay which are mixed with the machine oil, turpentine or other liquid in the same manner as the graphite. The use of these mixtures all give blanks which are clearer and freer from pits than those secured in the procedure heretofore practiced in which dry powdered materials were used to prevent the blanks from sticking to their supports. The greater freedom from pits is apparently due to the absence of any bunching of the powdered material such as occurs where such a material is applied dry to the supports for the blanks.

What I claim is:

1. A process of making optical disks from rectangular glass blanks which consists in coating one of the large faces of each of the blanks with a mixture comprising a finely

divided refractory material and a liquid subject to oxidation on heating to a high temperature, heating the blanks until they are plastic while supported on said coated faces and then pressing them into disk form in 70 molds.

2. A process of making optical disks from rectangular glass blanks which consists in coating one of the large faces of each of the blanks with a mixture comprising graphite and a hydrocarbon liquid, heating the blanks until they are plastic while supported on said coated faces and then pressing them into disk form in 75 molds.

3. A process of making optical disks from rectangular glass blanks which consists in coating one of the large faces of each of the blanks with a mixture comprising graphite and a liquid subject to oxidation on heating to a high temperature, heating the blanks until they are plastic while supported on said coated faces and then pressing them into disk form in 80 molds.

4. A process of making optical disks from rectangular glass blanks which consists in 90 coating one of the large faces of each of the blanks with a mixture comprising graphite and a hydrocarbon liquid carrying the blanks upon metal supporting means with their coated faces in contact therewith through a heated area and bringing them to a plastic condition, and then removing the blanks from said supporting means and pressing them into disk form in 95 molds.

5. A process of making optical disks from 100 rectangular glass blanks which consists in spraying one of the large faces of each of the blanks with a mixture comprising graphite and a hydrocarbon liquid, heating the blanks until they are plastic while supported on said coated faces and then pressing them into disk form in 105 molds.

WILLIAM W. POUNDSTONE.

110

115

120

125

130